

## UNITED STATES PATENT OFFICE

2,231,168

STEAM CYLINDER OIL AND PROCESS OF  
PREPARING THE SAME

Arthur Lazar, Berkeley, and Joseph V. Crenna,  
Concord, Calif., assignors to Tide Water Asso-  
ciated Oil Company, San Francisco, Calif., a  
corporation of Delaware

No Drawing. Original application June 11, 1937,  
Serial No. 147,784. Divided and this applica-  
tion February 2, 1939, Serial No. 254,310

3 Claims. (Cl. 252—39)

This invention relates to the treatment of lub-  
ricating oil to insure stability under condi-  
tions of high temperatures and pressures in the  
presence of steam and has for a particular ob-  
ject the preparation of a lubricating oil espe-  
cially adapted to function in the cylinders of  
steam engines.

In the manufacture of steam cylinder oils cer-  
tain specifications must be strictly adhered to be-  
cause of operating conditions peculiar to the uses  
of such oils.

Steam cylinder oils may not be supplied to the  
walls of the pistons and cylinders of the engine  
in many of the well-known forms of lubrication,  
but are introduced to the cylinder with the steam  
in such fashion that they are finely divided by  
atomization, whereby they are spread evenly  
over the moving parts.

In the modern steam engine practice the tem-  
perature of the steam in the cylinder of the en-  
gine when closed by the piston goes as high as  
500° F., under its corresponding pressure, and  
under such conditions it is highly important not  
only that a proper distribution of the oil is as-  
sured, but also that the stability of the oil is such  
as to resist decomposition, whereby undesirable  
deposits, such as coke, and the like, are elimi-  
nated.

Oils which have a tendency to emulsify with  
steam are best suited for steam cylinder oils and  
heretofore it has been common practice to com-  
pound with a mineral oil a certain percentage of a  
fatty oil, such as tallow, which causes emulsi-  
cation. Such fatty oil, or oils, usually represent  
up to 8% to 10% of the mineral oil, but in ad-  
dition to being costly, are decomposed at high  
temperatures which do not affect the mineral  
oil hydrocarbons, thus forming free fatty acids  
which attack metals under such temperature  
conditions.

The problems of steam cylinder lubrication are  
thus inherently different from the problems of  
lubricating the cylinders of internal combustion  
engines, due to operating conditions at high tem-  
peratures and pressures in the presence of water  
vapor, which factors require that the cylinders  
be preferentially wet with the oil rather than  
with the water.

For this reason, high viscosity oils have been  
found best suited for steam cylinder lubrication  
and such oils should be processed for emulsifica-  
tion with the steam used in order to provide the  
desired preferential wetting of the cylinder with  
oil.

Although high viscosity oils are generally ap-  
plicable to steam cylinder lubrication, this factor  
is not necessarily limiting as the invention in-  
volves the preparation of an oil which will pro-  
vide adequate lubrication while possessing an in-  
herent quality of stability under severe condi-  
tions of high temperature and in the presence  
of steam.

This invention provides a way of insuring the  
stability of steam cylinder oils while emulsifying  
the same under operating conditions, which is  
preferably accomplished in the following man-  
ner.

As a base stock for steam cylinder oils it is pre-  
ferred to select a lubricating oil which is com-  
posed mainly of saturated hydrocarbons, such  
oil, for example, being an asphaltic base, or  
mixed base, oil, which is highly refined by treat-  
ment with liquid sulphur dioxide, as in the well-  
known Edeleanu process, to remove unsaturated  
hydrocarbons, aromatics, etc. Such lubricating  
oil, thus treated, shows the greatest stability un-  
der high heat conditions, but, of course, a body  
of saturated hydrocarbons may also be prepared  
by extensive sulphuric acid treatment, or even  
distilled from certain stocks, such as Pennsyl-  
vania crudes.

It has been found, however, that certain oils  
of less saturated character can be stabilized by  
the processing method herein described. Such  
oils may include distillates from asphaltic or  
mixed base crudes, as well as lubricating oils ob-  
tained from such distillates by comparatively  
mild refining operations, such as the conven-  
tional acid treatment.

To the base lubricating oil is added a poly-  
valent metal soap, as lime or magnesium soap,  
of an organic acid, such for example as oleic acid,  
stearic acid, palmitic acid, naphthenic acids, or  
sulphonic acid, the proportion of such added soap  
ranging from very small percentages of the oil,  
e. g., .01% to 1% up to the limit of solubility of  
said soap in said oil.

The alkaline earth metals, calcium, strontium,  
barium, and magnesium, yield soaps with organic  
acids which exhibit suitable stabilizing qualifica-  
tions. When such soaps of a stable nature are  
added to oils, the resistance of the lubricant to  
decomposition, particularly under the high tem-  
peratures encountered in steam cylinder lubri-  
cation and other services, is greatly improved,  
and as a feature necessary for steam cylinder lu-  
brication we again emphasize the necessity of a

stable compounded lubricant as heretofore outlined.

We have found that the alkaline earth metal soaps do not form incrustations in service and of these calcium and magnesium soaps are preferred for economical reasons. However, the soaps of cadmium, aluminum, zinc, lead, copper, chromium, manganese, iron, cobalt, nickel, tin and mercury, may also be used.

10 Any organic acid which will yield a polyvalent metal soap with suitable stabilizing properties, is applicable to the process. Fatty acids, for example, oleic, stearic, palmitic, and derivatives of the same, have been successfully employed. Of 15 the fatty acids we prefer to use those of fourteen or more carbon atoms. Normally the more saturated acids, as stearic and palmitic, yield soaps which are less soluble in oil than the unsaturated acids, e. g., oleic, but a saturated acid of excellent 20 solubility may be obtained through the hydrogenation of unsaturated acids of certain types. To illustrate, unsaturated acids from fish oil when hydrogenated, yield acids which can be made into polyvalent metal soaps having superior 25 oil solubility properties. The acids from fish oils may be obtained in large quantities by splitting the esters normally present therein.

Polyvalent metal soaps of the hydrogenated acids derived as above described are soluble in 30 oil up to 5 per cent by weight, and are very efficient stabilizing agents.

Sulphonic acid soaps are very soluble in oil. Acids of this type which have been found particularly suitable, may be derived from the sulfonation of 30 to 200 seconds, Saybolt Universal 35 @ 100° F., oils of asphaltic origin, or raffinates derived therefrom by the well known Edeleanu treatment with liquid sulphur dioxide. Also from the extracted portion of the Edeleanu treatment aromatic type sulphonic acids may be prepared, from which suitable polyvalent alkaline earth or other metal aromatic sulphonic acid soaps can be made for the described purpose.

40 Polyvalent metal soaps of the naphthenic acids 45 are normally more oil soluble than those of the fatty acids, and are excellent stabilizing and emulsifying agents. Of the naphthenates those of calcium, magnesium, tin, and aluminum are preferred.

50 Depending largely on the degree of emulsification and the stabilizing influence desired, the content of soaps dissolved in the oil may vary from a minute amount up to the limit of oil solubility. The following table is illustrative of the 55 solubilities of the calcium soaps in the oil.

TABLE I

|                          | Solubility in paraffine oils | Solubility in oils of asphaltic origin |
|--------------------------|------------------------------|----------------------------------------|
| Calcium sulphonate.....  | 50% or more.....             | 50% or more.....                       |
| Calcium naphthenate..... | 4% max.....                  | 10% max.....                           |
| Calcium oleate.....      | 0.5% max.....                | 1% max.....                            |
| Calcium stearate.....    | 0.2% max.....                | 0.4% max.....                          |
| Calcium palmitate.....   | 0.1% max.....                | 0.3% max.....                          |

The above soaps are listed in the order of:

Decreasing solubility in oil,  
Increasing qualifications as lubricant stabilizers,

70 Decreasing emulsifying properties.

A table similar to the above can be prepared for magnesium soaps which have similar properties to the respective calcium soaps except they are in general slightly more soluble in oil and not 75 quite as stable.

Aluminum soaps of organic acids show excellent solubility in mineral oils of all types. However, when added in percentages in excess of about 2%, the compounded oils possess a stringy structure, which for our purposes is undesirable. 5 The preferred range for aluminum soaps is between 0.01% up to 1.0% by weight of the oil.

In the preparation of lubricants we have also found that the solubility of the less soluble polyvalent metal soaps can be increased by the mixing therewith of a more soluble soap of polyvalent metals. For example, the solubility of calcium oleate can be tremendously increased by the simultaneous incorporation in the lubricant of a comparatively small percentage of a more soluble calcium or other polyvalent metal soap, such as calcium naphthenate or calcium sulphonate. This is a particularly important feature when it is desired to permanently incorporate in the oil soaps of relatively low solubility. The following 20 table clearly illustrates this feature, and it should be noted that the solubility of calcium oleate in the same oil and under the same conditions has been increased manyfold by the addition of a 25 small percentage of a more soluble soap.

TABLE II  
*Solubility of calcium oleate in California lubricating oil*

|                                               | Per cent |
|-----------------------------------------------|----------|
| Calcium oleate.....                           | 1.0      |
| Calcium oleate + 10% calcium naphthenate..... | 2.5      |
| Calcium oleate + 20% calcium naphthenate..... | 4.0      |
| Calcium oleate + 30% calcium naphthenate..... | 7.0      |

Although in the above example calcium naphthenate has been shown because of its well known oil solubility feature, this in no way should be indicated as a limitation on this feature, and a similar result is obtained by the use of other more soluble soaps, such as the polyvalent metal soap 40 of sulphonic acid.

In describing this invention which is particularly directed towards the manufacture of a steam cylinder oil of stable oil and soap characteristics, it is important that a permanent solution of soaps be incorporated in the oil. Therefore, in order to increase the total soap content for this or other possible lubrication purposes, it has been found advantageous to utilize stable soaps made from a mixture of acids.

In order to provide the maximum stability to 50 resist the high temperature conditions encountered, and still provide enough soap for proper lubrication in conjunction with steam or otherwise, such emulsifiable oil should contain a maximum quantity of the preferred soaps described herein.

The novel feature of mixing two or more soaps is utilized when it is desired to increase the solubility of the more insoluble polyvalent metal soaps in oil over the maximum noted in Table I.

The following table is illustrative of the quantities of polyvalent metal soaps normally added to the oil and the preferred range of soap content for the steam cylinder oils.

TABLE III

|                   | Range                   | Preferred range           |
|-------------------|-------------------------|---------------------------|
| Sulphonates.....  | Percent<br>Up to 5..... | Percent<br>0.01 to 2..... |
| Naphthenates..... | Up to 5.....            | 0.01 to 1.0.....          |
| Oleates.....      | Up to 1.0.....          | 0.01 to 0.1.....          |
| Stearates.....    | Up to 0.8.....          | 0.01 to 0.1.....          |
| Palmitates.....   | Up to 0.3.....          | 0.01 to 0.1.....          |

It is important in the application of the above ranges of soap content to lubricants to add just sufficient soap to give the desired stabilization properties. In steam cylinder oils the addition is such as to give the desired emulsifying properties and prevent the formation of incrustations or deposits on the cylinder walls of the lubricated mechanism. In general the addition is so small that the amount of ash arising from its use as an emulsifier is too small to be determined analytically.

The use of soap results in a steam cylinder oil of unimpaired stability which emulsifies sufficiently to get the desired distribution, the soaps being easily combined with the saturated hydrocarbons, due to their oil solubility.

Likewise, a steam cylinder oil having the required emulsifying properties may be prepared from oils which result from the distillation of a suitable crude stock and which may be naturally composed mainly of saturated hydrocarbons. For instance, residual oils of Pennsylvania origin when traces of oxides, or hydroxides, are added to the oil when heated, such oil develops the desired pronounced emulsifying properties. To such oils, an organic acid or acids not normally present in petroleum may be added, and the requisite amount of polyvalent metal oxide or hydroxide, to accomplish substantial neutralization of the oils, applied.

A preferred amount of polyvalent metal oxide or hydroxide, for example, magnesium oxide, or lime, or other alkaline earth oxide, or hydroxide, which may be added to such residual oil varies from 0.01% to 0.1%, and such is incorporated in the oil by intimate mixing at elevated temperatures, preferably about 300° F., and generally in excess of atmospheric temperatures. This oil may then be used as straight steam cylinder oil, or may be blended in amounts of from 10% to 20% with a body of a highly refined oil of high stability, such as the SO<sub>2</sub> treated oil previously described.

The soaps may be added directly to the oil, during agitation either mechanically or with air, and the oil heated to 200—300° F. The preferred method however, is to first dissolve the desired quantity of organic acid in the oil and slowly add a metallic oxide or hydroxide, of the polyvalent metals previously cited, heating preferably to about 300° F., and generally in excess of atmos-

pheric temperature, and agitating the mixture until neutralization of the free acid is substantially complete. In such manner the soap is more readily incorporated in the oil and excellent distribution and dispersion of the soap in the oil is accomplished. When prepared in this manner with excess quantities of acid and oxide the quantity of the soap which is retained in the oil represents the maximum of solubility. This oil may be used as is, or blended in amounts from 10% to 50% with additional quantities of suitable base oils.

While it is unnecessary, the use of small amounts of an acidless fatty oil with the steam cylinder oils prepared as above described, has sometimes a beneficial effect in lowering the surface tension, but the quantity used, from 0% to 3% is kept as low as possible and in any event is far less than the amount normally used in compounding steam cylinder oils.

This application is a division of our copending application Serial Number 147,784 filed June 11, 1937 which is a continuation in part of our copending applications, now Patents Nos. 2,084,531-2, dated June 22, 1937.

We claim:

1. A steam cylinder oil consisting mainly of saturated hydrocarbons substantially devoid of free organic acids, and containing a small percentage of a polyvalent metal soap of comparatively low solubility with a still smaller percentage of a more soluble polyvalent metal soap, the total percentage of the soaps being insufficient to leave an appreciable deposit of ash when the mixture is injected into the cylinder of a steam engine.

2. The method of increasing the solubility of a relatively low soluble alkaline earth metal soap such as calcium oleate, in a steam cylinder lubricating oil, which consists in incorporating with the oil and soap a more soluble alkaline earth metal soap, such as calcium naphthenate, in amount less than the less soluble soap, the total amount of the two soaps together being between .01% and 1% of the weight of the oil.

3. A lubricating oil containing up to one percent of a soap mixture consisting of calcium oleate and calcium naphthenate, the naphthenate being less than 40% of the weight of the oleate.

ARTHUR LAZAR.  
JOSEPH V. CRENNAN.